

Feb. 21, 1956

F. NIELSEN

2,735,147

GATING SYSTEM FOR CASTING METALS

Filed Jan. 9, 1953

2 Sheets-Sheet 1



*Fig. 1*



*Fig. 3*



*Fig. 2*



*Fig. 4*



*Fig. 5*



*Fig. 6*

INVENTOR

*Friedrich Nielsen*

BY *Bailey, Stephens & Huettig*  
ATTORNEYS

Feb. 21, 1956

F. NIELSEN

2,735,147

GATING SYSTEM FOR CASTING METALS

Filed Jan. 9, 1953

2 Sheets-Sheet 2



*Fig. 7*



*Fig. 8*



*Fig. 9*

Friedrich Nielsen

BY  
Bailey, Stephens & Huettig  
ATTORNEYS

1

2,735,147

## GATING SYSTEM FOR CASTING METALS

Friedrich Nielsen, Muhlacker, Germany

Application January 9, 1953, Serial No. 330,479

Claims priority, application Germany October 31, 1949

3 Claims. (Cl. 22—134)

This invention relates to the casting of metals. In particular, the invention is directed to a gating system for pouring molten metal, especially light metals, into a mold.

This invention is a continuation-in-part of my application S. N. 261,956, filed December 17, 1951, for "Casting Metals," now abandoned.

In recent years the art of pouring molten metals has been increasingly interested in the technique of the so-called gating practice in which the molten metal is poured from a ladle into a pouring runner from which it flows through a gate into a mold. Heretofore the design of the system has most frequently been based on the cross-sectional ratio between the runner inlet, the runner, and the gate outlet from the runner, as for example 4:3:2, or 10:9:5, or 100:95:90, or 3.6:4:2. These numerical proportions merely approximate the dimensions of a pouring runner in which the cross-section is narrowed from the inlet to the outlet gate so that the velocity of flow of the molten metal is not sensibly impeded by the runner. Whatever advantages which may be obtained from such system are offset by the fact that the velocity of the metal entering the mold creates eddys and flow shocks in the casting which are very detrimental to the same.

In order to avoid disturbances of the metal in the mold, it has been proposed to slow the velocity of the metal in a straight runner by progressively, in steps, widening the way from the inlet through the runner to the gates as for example in the ratio of 1:2.5:10. However, although the principle of diminished velocity to produce laminar flow at the gate is met, in actual practice the runner became so wide adjacent the gate as to permit the formation of slag and oxide skins on the very large exposed surface of the slowly flowing molten metal. In addition, a uniform flow cannot be maintained at the gate in the beginning of the casting as the molten metal does not entirely fill the wide runner adjacent the gate.

The objects of this invention are to produce a casting system in which both the exposed surface area of the molten metal and the velocity of discharge into the mold are kept to a practical minimum; to produce a runner in which the kinetic energy of the molten metal received from a ladle is dissipated substantially before the metal is discharged through the gate; and to produce a runner by means of which a steady, quasi-laminar flow of metal into a mold is obtained.

In general, these objects are obtained by constructing a covered runner having a plurality of straight sections connected to each other by sharp bends and which widens from the inlet to the outlet gate. Preferably the runner has right angle turns so that as the metal flows around each turn there is an impact loss of energy and a corresponding decrease in velocity. Each successive section between bends is proportionately increased in width and cross-sectional area so that a uniform volume of flow is maintained through the runner. Consequently, the molten metal can be discharged from the runner at a velocity which will not cause disturbances in the mold,

2

and at the same time the cross-section of the runner is kept small enough so that the surface of the metal will not oxidize to an objectionable extent.

The invention is described more fully with reference to the accompanying drawings in which the invention is illustrated diagrammatically.

Figure 1 is a front view of a runner system according to the invention, a portion being shown in section on the line 1—1, Fig. 2;

10 Figure 2 is a plan view of the invention shown in Fig. 1;

Figure 3 is a front view of a modified form of the invention, partly shown in section on the line 3—3, Fig. 4;

Figure 4 is a plan view of the invention shown in Fig. 3;

Figure 5 is a front view of a third form of the invention, shown partly in section on the line 5—5, Fig. 6;

Figure 6 is a plan view of the invention shown in Fig. 5;

Figure 7 is a front view of a fourth form of the invention;

Figure 8 is a cross-sectional view on the line 8—8, Fig. 7; and

20 Figure 9 is a graph showing the range in which the invention can be practiced.

In Figures 1 to 8, the invention is described for a gating system in which the runner sections are connected at 90° angles. For other angles the ratios are shown in Figure 9.

As seen in Figs. 1 and 2, the runner 10 is provided with an inlet 12 through which molten metal is received from a furnace, or ladle, and with outlet gates 14 through which metal flows into a mold 16.

30 Runner 10 has a course including sharp abrupt bends between the inlet and the gates. Channel section 16, adjacent inlet 12, is narrow and is joined to section 18 of greater width by a right angle turn. Section 18 similarly joins section 20, which likewise is continued into section 22 and gates 14. In the diagrammatic drawings the slope of the channel and the slight rounding of the corners according to conventional practice are omitted.

35 Molten metal enters the runner through inlet 12 with a velocity determined by the height of metal in the inlet. The flow of molten metal on being deflected into section 18 suffers an energy loss, and as the flow of metal is briefly and successively deflected into channels 20 and 22, and out through gates 14 the velocity of flow is diminished further.

40 In deflecting the flow of metal through an angle of 90°, the impact energy loss causes about a 37.5% reduction in velocity, the flow into the succeeding channel amounting to 62.5% of the original velocity. Consequently, in order to maintain a uniform volume of flow, the new channel section must have a cross section increased about

$$\frac{100}{62.5}$$

55 or 1.60 times the cross-section area of the first channel section. Thus, channel section 18 has a cross-sectional area 1.6 times that of channel 16, and sections 20, 22 and gates 14, respectively each increased over the preceding section. Each section need only be long enough to obtain the desired deflection and energy loss, and each section has a length as short as permitted by runner construction, a length of a few centimeters usually being sufficient. The inner corners of the channel may be slightly rounded in order to maintain good flow characteristics, but the outer corners should be kept as sharp as possible in order to gain the maximum impact energy loss.

60 It is practical to work with smaller ratios for the stages of widening the channel sections, as for example 3:4=1.33, which corresponds to about a 25% velocity reduction in each stage. Any residual small static excess

pressures remaining from a preceding stage can be corrected for if harmful. The range of ratios usable for 90° bends is from 1:1.01 to 1:1.60, note Figure 9.

The following specific example is given for runner formed as in Figures 1 and 2, it being assumed that a velocity loss of 29.3% is desired in each channel section.

|                                | Channel Section |     |     |     |      |
|--------------------------------|-----------------|-----|-----|-----|------|
|                                | 16              | 18  | 20  | 22  | 14   |
| Cross-sectional area (sq. mm.) | 100             | 141 | 200 | 283 | 400  |
| Pressure Head (cm.)            | 32              | 16  | 8   | 4   | 2    |
| Velocity—cm./sec.              | 250             | 177 | 125 | 88  | 62.5 |

The cross-sectional area given for gates 14 represents the combined areas of the several gates.

It can be seen from the above table that the static pressure head at the gates is only in the order of a few centimeters, and this head will not increase as pouring takes place. A calm filling of the mold is thus ensured throughout the pouring operation.

While in Figures 1 and 2 the channel sections are shown of equal height, but of varying width, the height can be also varied as shown in Figures 3 and 4, this sometimes being desirable in order that the runner can be adapted to the shape of a mold and the position of the gates with respect thereto. In Figures 3 and 4, from inlet 30, channel sections 32, 34, 36 and 38 are of progressively decreasing height, and increasing width, including gate 40, from which metal is discharged into mold 42. Furthermore, the loss of energy impact effect is increased by extending each channel section slightly beyond the connection with the succeeding section as shown at 33, 35, 37 and 39.

Special provision can be made for the collection of slag or oxide formations as shown in Figures 5 and 6. From inlet 50, channel sections 52, 54, and 56 as well as gates 60 are designed as described for Figure 1, metal flowing to mold 62. One or more channel sections can be formed as a slag collector, preferably the next to the last stage as section 58. This section is higher than the preceding sections so that the slag floating on top of the molten stream will collect. Normally, the cross-sectional area of the collecting section should be in conformity with its place in the sequence of sections. It may be larger if the preceding and succeeding sections are in proper ratio, for example, as 1:2 when the step ratio is 1:1.41; or 1:1.77 if the ratio is 3:4. In such enlarged sections, additional energy losses may occur due to direction changes and impact losses, and such must be allowed for in the design of the entire system.

In Figures 7 and 8, the system is applied to the casting of vertical molds, and also illustrates the use of branched channel sections. Molten metal flows vertically downward in inlet 70, then horizontally through channel section 72, then vertically through section 74. The channel is then split into branches 76a and 76b, the combined area of which equals the value necessary to maintain the sequential ratio adopted for the system. Branches 76a and 76b serve as distribution channels serving gates 80 from which metal is discharged into molds 82. Where more than one gate exists for one branch, as shown, the channel branch section is narrowed, as at 77a and 77b, adjacent the outermost gate in order to maintain equal fluid pressures at all the gates.

The system of Figures 7 and 8 ensures the correct feeding of metal to a plurality of similar molds, or to various inlets into a large casting, with a reliability greater than heretofore obtainable. Unequal feeding through a plurality of gates is virtually eliminated.

Branched section channels can also be used in the horizontal casting systems of Figures 1 to 6. The sections may be branched, and subsequently united without

the risk of causing the metal to eddy or froth if done when the metal has reached a low velocity section.

If, in a vertical casting, the mold is so large as to require the use of lateral gates, the sum of all the gate areas may exceed the established ratio because the gates come into operation one after the other. Thus the last distribution channel can be increased beyond the ratio as the low velocity has already been achieved in the preceding channel sections. In the case of very large molds, the use of lateral gates is to be recommended in view of the low rising speed of the metal. Even in horizontal castings it is sometimes advantageous to have the channel sections gently sloped upwards toward the gates when a particularly low discharge speed is desired.

In Figure 9, the graph illustrates the range of angles and ratios in which the invention can be practiced. The limits for an angle of 20° are ratios from 1.05 and 1.2. The limits for an angle of 150° are ratios from 1.3 and 2.5. The upper curve AB and the lower curve CD define the area within which the system successfully operates. Above the curve AB, the ratios produce a system in which foaming occurs in the runner system, while below curve CD, the ratios produce eddy currents and slag in the mold. Preferably, in the ordinary case, the ratios employed are those in the area lying in the upper half of the middle third between curves AB and CD.

The simplest system is to have 90° connections between the runner sections. However, it is desirable at times to use other angles, or combinations of other angles in the system. This is determined by the way the mold is situated, the shape of the casting and other factors. For example, where very high inlets are used, it is desirable to use angles less than 90° in the beginning of the system because the reaction pressures on the walls of the runner are small, and the runner sections are saved from wear. In general, the energy losses increase as the angles increase. Where combinations of angles are used, the ratio of increase in cross-section permissible in the system can be selected from Figure 9.

The principles of the invention are also applicable to the normal poured casting where the metal is simply poured into the top of a mold, and to pressure casting, as the maintenance of a smooth quasi-laminar flow of metal devoid of gas, bubbles, and eddy disturbances, inherently produces a superior casting.

Having now described the means by which the objects of the invention are obtained, I claim:

1. In a gating system, a molten metal pouring runner having an inlet end and a discharge gate, further comprising communicating channel sections joined to each other and forming a runner having a plurality of angles to effect a loss in kinetic energy in metal flowing through said sections to said discharge gate, each channel section between said inlet end and said discharge gate being successively increased in cross-section in a ratio lying between the curves AB and CD in Figure 9 of the drawings.

2. In a gating system as in claim 1, the height of said channel sections being progressively decreased from said inlet end to said discharge gate.

3. In a gating system as in claim 1, one of said sections being branched with the sum of the cross-sectional areas of the branches being equal to the cross-sectional area required for the sequential position of said branched section in said runner system.

#### References Cited in the file of this patent

#### UNITED STATES PATENTS

- 1,553,628 Norton Sept. 15, 1925  
 2,219,012 Kirby Oct. 22, 1940  
 2,629,647 Arnette Nov. 14, 1950

#### OTHER REFERENCES

- Pages 68 to 73, inclusive, and 252, The Foundry, October, 1948.